# EUROPEAN PATENT SPECIFICATION

(11) **EP 0 043 999 B1**
(45) Date of publication and mention of the grant of the patent: **29.01.1986**
(21) Application number: 81105149.9
(22) Date of filing: 02.07.1981
(51) Int. Cl.: B22D 19/16, B22D 13/02

(54) **A method of centrifugally casting a metal casting**
Verfahren zum Zentrifugalgiessen eines metallischen Gussstückes
Procédé pour la coulée par centrifugation d'une pièce en métal

(30) Priority: 14.07.1980 US 168728
(43) Date of publication of application: 20.01.1982
(73) Proprietor: ABEX CORPORATION, Stamford, Connecticut 06904-2268 (US)
(72) Inventor: Khandros, Igor Y., Hoboken, N.J. 07030 (US)
(74) Representative: Hansmann, Axel, Dipl.-Wirtsch.-Ing.

## Description

The invention relates to a method as set out in the preamble of claim 1.

Such a method is described in DE-C-566 714. In the castings obtained by this known process the metal to be poured first will have the physical and chemical properties which are desired for the exterior layer of the hollow body. That means a casting comprising e.g. a chromium or chromium-rich outer zone and an aluminium or aluminium-rich inner zone will be obtained by first pouring chromium or the chromium containing alloy and then the aluminium or aluminium containing alloy so that the latter will be in contact with the ambient air and therefore prone of being oxidized.

The object of the present invention is to produce a centrifugally cast tube of a heat-resistant alloy high in content of a relatively light and relatively low melting, easily oxidized metal, e.g. aluminium, in the inner zone while nonetheless producing a casting free of objectionable dross and oxide inclusions, and to be able to produce at will gradients of concentration of the oxidizable metal in the cross section of the casting, or, in a broader sense, to cast an alloy containing a light and low melting, easily oxidized metal centrifugally while protecting said lighter metal from being oxidized.

This problem is solved by the method of the claims.

Aluminium oxidizes easily when attempted to be cast simultaneously with the metal which is to alloy. The present method may use aluminium in a heat-resistant alloy which has chromium and one can displace some of the chromium with aluminium.

The purpose of pouring the low melting point, easily oxidized metal first and allowing it to solidify while afterwards melting it with higher melting point base metal is that it will not deposit impurities or leave porosities inside the cast tube since it cannot oxidize internally. There is only a thin layer of dross or oxide at the inside diameter of the tube when the method is completed, and the layer is only superficial and easily removed by grinding or abrading which is usually done conventionally to produce a tube with a clean or bright inside surface.

In the drawings:
Figures 1, 1A and 1B are sectional views, partly. schematic, of a centrifugal mold in several stages of producing a casting and wherein, for convenience, the ordinary end caps for the mold are omitted;
Figure 2 is a photomicrograph (magnification 6x) of a cross section of a tube cast centrifugally in accordance with the present invention;
Figure 2A is a graph in which the abscissa is substantially aligned to and shows the distribution of elements across the radius of the casting of Figure 2;
Figure 3 is a photomicrograph of the casting of Figure 2 at a magnification of 40x; and
Figures 4 and 4A are views similar to Figure 1 showing several stages of casting centrifugally under another embodiment of the invention.

Typical centrifugal mold apparatus is shown in Figure 1 comprising a centrifugal mold 10. The molten metal for the casting pours from the end of a spout 13A which is part of a pouring vessel 13. Because of the rotating mold the entrant metal, whatever its kind, spirals down the inner diameter ID of the mold, as the molten metal will act like any other free body of liquid seeking its own level, especially with the force of the reservoir (vessel 13) behind it.

Earlier in the process, a light, low melting point metal 12 was deposited in the same way on the ID of the mold, having solidified, and as shown in Fig. 1 a heavier metal 14 having a much higher melting point is being deposited on the previous layer of lighter metal 12.

The first portions of heavier metal 14, therefore, will remelt outer layers of the lighter metal 12 and will spirally slip across the partially remelted substrate of the lighter metal like a skate on ice. The oncoming streams of the high melting point metal gradually remelt remaining light metal and the rest of the heavier metal eventually slips over the molten alloy containing both heavier and lighter metal. At these moments the lighter metal is dissolved only in the outside diameter (OD) adjustment zone of the molten tube and, therefore, this zone is lighter than the rest of the metal. Because of centrifugal force, the heavier metal 14 will gravitate in the direction of the outside (OD) diameter of the centrifugal mold, or stated in other words, the lighter metal will be at the ID of the resultant cast tube T.

Essentially, there are four stages in principle although in actual practice they may by no means exhibit the distinctiveness shown in the drawing. The first stage is solidification of the light metal followed next by the occurrence of the heavier, high melting point spiralling across the earlier deposited light metal, Fig. 1. The taper shown for the lighter metal in Fig. 1 is actual, and is desirable in some cases for the achieving of a uniform ID alloyed layer, especially when a lower rotating speed of the mold is employed. In the third stage the melted metals attain uniform wall thickness with the heavier metal at the ID, but because the mold continues to rotate the heavier metal moves to the OD, Fig. 1 B, where it remains while the casting cools to the solid state during the last stage.

More specifically, a No. 356 aluminum alloy (6.5 to 7.0% silicon) was poured at 1450°F (785°C) into the rotating mold which had been preheated to 400°F (203°C). Afterwards, a heat-resistant alloy (HRA alloy) of 35% nickel, 19% chromium, 0.42% carbon, 1.2% silicon and 1.2% manganese (balance iron except for impurities) is poured at 2900°F (1580°C) onto the earlier formed, thin aluminum "tube" 12 from the same end of the mold.

The resultant centrifugally cast tube is found to contain three zones of metal:
(1) an ordinary HRA zone at the outside diameter with some residual AI dissolved in it,
(2) a transition zone, and
(3) an aluminum-rich alloy zone at the inside diameter, all zones being shown in Figs. 2 and 3, as will be explained in more detail below.

Aluminum oxide clusters were observed only near the inside diameter (ID) surface of the tube, and in surprisingly small quantities for an air- melted heat-resistant tube containing so much aluminum.

The three zones (1), (2), and (3) are designated in Figs. 2 and 3. The OD for the most part is the HRA alloy identifed above but containing evenly distributed aluminum nitrides while the aluminum-rich alloy at the ID contains Fe-Ni-AI with some chromium carbides precipitated in intermetallic phases precipitated in interdendritic areas.

Clearly, when the heavier metal 14, Fig. 1, was poured the standard HRA melt covered and remelted the aluminum alloy which was then shifted toward the inside diameter during continued rotation of the mold. However, some aluminum is dissolved in the HRA alloy during the shift, lowering the melting point of the alloy at the OD. The greater alloying with aluminum occurs at the ID, lowering the melting point of that alloy still further. The ID may be covered by an aluminum-rich oxide film providing protection against further oxidation. Those light oxide inclusions which get underneath the film do not propagate deeply into the metal owing to their light weight and the centrifugal force.

Because of the increase in aluminum content a tube cast centrifugally in the manner of the present invention will exhibit higher corrosion, oxidation and carburization resistance compared to the corresponding HRA alloy having no aluminum. Also, the aluminum-rich layer at the ID, having heavy precipitation of intermetallic phases and carbides will be harder and will exhibit improved abrasion resistance for those applications where hardness is a controlling factor. The hardness measured at the ID surface of several tubular products produced according to the present invention was up to 430 BHN.

In any event, the process of the present invention may permit reduction in chromium content relying on aluminum substitution, especially for those applications where high temperature corrosion and oxidation resistance are most needed.

The HRA alloy specified above is only one of a whole host to which the invention may be applied. A family of HRA alloys to which the present invention may be applied is given in Patent No. 4,077,801:

Most of aluminum alloys may be employed without difficulty, depending on the final composition of metal required. Additions of other easily oxidized elements, such as titanium or boron, can be placed into the metal 12 in the form of a course powder of their low melting temperature alloys.

When additions of surface active elements such as boron are employed the time of solidification of the casting is apparently reduced due to lowering of the surface tension between the solid state nuclei and liquid phase. As a consequent, less centrifugal separation was observed and almost uniform distribution of aluminum through the wall of the casting resulted.

The principles of the invention would be equally applicable when replacing the HRA alloy with any steel such as a stainless steel, any other HRA alloy, or a nickel or cobalt base alloy; indeed the replacement can be any alloy melting appreciably higher and which is appreciably heavier than the light weight alloy and which is advantaged or improved by having the light weight, low melting point metal move therethrough while both are in the molten state.

Preferably the mold will be preheated at 350°F-400°F (175°C-203°C) to avoid premature solidification when the lower melting point metal is first introduced to the mold cavity. Since the mold in most instances will have a mold wash lining (e.g. 1,57 mm that is one sixteenth of an inch thick) on the inside diameter derived from a mixture of silica and water, heating the mold to drive off the water will also afford all, if not the major part of the preheat.

For any given amount of lighter, low melting point metal initially poured the distribution of the lighter element through the cross section of the casting will be proportional to the following major influences:
(1) The rotational speed of the mold over the time period required for solidification to be attained because a higher speed means higher degree of centrifugal separation and more of the heavier metal moving radially outside; higher rotational speed will also result in higher longitudinal velocity of the heavier metal, so that less heat is lost during this period of the process and, therefore, more time is available for the centrifugal separation;
(2) The pouring temperature of the heavier metal, because when the metal is poured "hotter", the total time of solidification is increased and more centrifugal separation occurs; and because metal possesses higher fluidity at higher temperatures it will move more quickly in the longitudinal direction in the first moments of the process;
(3) The thickness of the mold wash, because it also influences the total time of metal solidifications.

It will be recognized that alloying between the light and heavy metals takes place inside the mold. At all times the light metal, is prevented from doing so to any objectionable degree. The objectionable oxidation is that which ordinarily occurs when an HRA metal, combined with aluminum, is poured into the mold from a vessel as 13, at or above the melting point of the HRA-aluminum alloy. Objectionable oxidation does not occur when merely pouring the aluminum alloy at its melting point into a preheated mold, say when pouring at 1400°F (755°C) into a mold at 400°F (203°C). Now then, when the HRA metal 14, not yet alloyed with aluminium 12, is poured at say 2900°F (1580°C), the aluminum, though melting on contact, Fig. 1, is covered by the molten HRA metal which induces the melting, and hence the easily oxidized metal is blanketed against oxidation. In comparison, an HRA-aluminum alloy ofthe proportion specified above, when poured all at once, will exhibit a drossy, porous, heavily oxidized ID which can be rendered acceptable only at an exhorbitant machining cost to reduce the wall thickness to a radius of sound metal; the loss in yield is prohibitive in most instances.

A further advantage is the ability to pour the HRA metal 14 at a temperature lower than heretofore. Thus, the HRA metal or the high melting point metal is usually poured at a temperature considerably above the liquidus so it will not be solidified too quickly by the much cooler mold. Such is not necessary under the present invention, especially when the lighter metal is aluminum because in that case the aluminum not only melts, becoming a "lubricant", it is dissolved in the HRA molten metal at the same time and heat of solution is generated, meaning the HRA metal need not be poured at the higher temperature to assure sustained fluidity.

In accordance with thebroaaer objective of the invention it is possible to reduce further the formation of nonmetallic inclusions and improve the surface quality of the castings even at the ID. This is made possible by displacing air from the mold, after the light metal has solidified, with a confined body of non-oxidizing gas which itself is afterwards displaced as an incident to casting the heavy metal or alloy. Thus, referring to Fig. 4, a centrifugal mold 20 is provided with the usual end caps, but in this instance one end cap 22 is provided with one or more vent openings 24 and the other end cap 26 has a central aperture 26A of a size to admit a lance 28 which feeds a non- oxidizing gas such as argon into the mold interior after the light metal has solidified. Argon displaces air out the vent hole, which is continued until the body of gas inside the mold is the non-oxidizing gas. The lance is withdrawn and the openings in the end caps are temporarily sealed with a displaceable plug or rupturable diaphragm (not shown) which may be nothing more than a piece of plastic film.

When the casting is to be completed, the pouring spout 30 of a pouring vessel 32 is positioned in aperture 26A incidental to allowing molten metal 34 (heavy metal) to pour onto the previously poured light alloy at the inside diameter of the mold, which is being rotated.

The molten metal expands the gas (NG) which is forced from the mold at the vent 24 and at the annular venting space presented by aperture 26A.

The non-oxidizing gas continues to be displaced as the molten metal spirals down the mold, seeking its own level as any other fluid body.

Since the mold was and remains air-free from the inception of pouring the heavier metal there can be no appreciable oxidation of the molten metal, nor formation of nonmetallic inclusions at the ID.

## Claims

1. A method of centrifugally casting a metal casting, particularly a tube, comprising the steps of casting in succession two layers of metal of different density and of different melting points, whereby a transition zone between the two layers is established and the two layers are solidified to complete the centrifugally casting, characterized by pouring the light and low melting metal which, in addition, is more easily oxidized, onto the inside diameter of a rotating centrifugal mold (10) and allowing this metal to solidify in the mold (10) so that it has a thick section at one end of the mold (10), tapering to a thinner section; pouring the denser and higher melting metal initially onto the thick section of the solidified metal while rotating the mold (10), thereby gradually remelting the easily oxidized metal and progressing down the length thereof as a protective blanket for preventing oxidation of the easily oxidized metal at the pouring temperature of the denser metal; continuing rotation of the centrifugal mold (10) until the easily oxidized metal is entirely covered by the blanket and also until the easily oxidized light weight metal has moved radially inward through the denser metal to reach the inner diameter of the casting, whereby the easily oxidized metal has been prevented from undergoing objectionable oxidation, thereby obtaining a centrifugal casting having at and near the outside surface a zone (zone 1) having a high concentration of the denser metal alloyed with a low concentration of the easily oxidized, lighter metal; a zone (zone 3) having a higher concentration of the easily oxidized, lighter metal, higher than in zone (1), alloyed with a lower concentration of the denser metal, lower than in zone (1), located at and near the inside surface; and a transition zone (zone 2) between the zones (1 and 3) where the concentration of the easily oxidized, light metal is continuously increasing radially in the direction of the inside surface.

2. A method according to claim 1 in which the easily oxidized, light and low melting metal is aluminium or an aluminium alloy.

3. A method according to claim 1 or 2 in which the denser metal is a heat-resistant alloy consisting in percent by weight essentially of:

4. A method according to claim 1 in which the denser metal is selected from the group consisting of steel or cobalt base alloys or nickel base alloys or heat-resistant alloys containing both nickel and chromium.

5. A method according to claim 1 including the step between pouring the easily oxidized, light and low melting metal and pouring the denser metal of displacing air from the interior of the mold (10) with a nonoxidizing gas, confining the nonoxidizing gas to the interior of the mold (10), and providing for escape of the nonoxidizing gas when pouring the denser metal.

6. A method according to claim 5 in which the mold (10) has end caps (22) of which at least one is provided with a vent route (24) for the escape of nonoxidizing gas and including the step of sealing that vent route (24) to confine the nonoxidizing gas until the denser metal is poured.

## Revendications

1. Procédé de coulée par centrifugation d'un moulage en métal, en particulier un tube, comprenant les étapes qui consistent à couler successivement deux couches de métal ayant des masses volumiques différentes et des points de fusion différents, de manière à établir une zone de transition entre les deux couches et à solidifier les deux couches pour achever la coulée par centrifugation, caractérisé en ce qu'il consiste à couler le métal léger et à bas point de fusion qui, de plus, est plus aisément oxydé, sur le diamètre intérieur d'un moule centrifuge rotatif (10) et à permettre à ce métal de se solidifier dans le moule (10) afin qu'il comporte une section épaisse à une première extrémité du moule (10), s'effilant jusqu'à une section plus mince; à couler le métal plus dense et de point de fusion plus élevé, intialement sur la section épaisse du métal solidifié pendant que le moule (10) est en rotation, de manière à faire refondre ainsi progressivement le métal aisément oxydé, en progressant sur sa longueur, sous la forme d'une nappe protectrice destinée à empêcher l'oxydation du métal aisément oxydé à la température de coulée du métal plus dense; à poursuivre la rotation du moule centrifuge (10) jusqu'à ce que le métal aisément oxydé soit entièrement recouvert de la nappe et également jusqu'à ce que le métal aisément oxydé, de poids léger, se soit déplacé radialement vers l'intérieur à travers le métal plus dense pour atteindre le diamètre intérieur du moulage, le métal aisément oxydé ayant été ainsi protégé d'une oxydation critiquable, ce qui conduit à l'obention d'un moulage centrifuge présentant, à et à proximité de la surface extérieure, une zone (zone 1) ayant une concentration élevée du métal plus dense, allié à une faible concentration du métal aisément oxydé, plus léger; une zone (zone 3) ayant une concentration plus élevée du métal plus léger, aisément oxydé, supérieure à celle de la zone (1), allié à une concentration inférieure du métal plus dense, inférieure a celle de la zone (1), à et à proximité de la surface intérieure; et une zone de transition (zone 2) entre les zones (1 et 3) où la. concentration du métal léger, aisément oxydé, s'élevé en continu radialement dans la direction de la surface intérieure.

2. Procédé selon la revendication 1, dans lequel le métal léger, aisément oxydé et à bas point de fusion est de l'aluminium ou un alliage d'aluminium.

3. Procédé selon la revendication 1 ou 2, dans lequel le métal plus dense est un alliage résistant à la chaleur, constitué, en pourcentages en poids, essentiellement de:

4. Procédé selon la revendication 1, danslequel le métal plus dense est choisi dans le groupe constitué d'acier ou d'alliages à base de cobalt ou d'alliages à base de nickel ou d'alliages résistant à la chaleur contenant à la fois du nickel et du chrome.

5. Procédé selon la revendication 1, comprenant l'étape qui consiste, entre la coulée du métal léger, aisément oxydé, à bas point de fusion, et la coulée du métal plus dense, à chasser l'air de l'intérieur du moule (10) à l'aide d'un gaz non oxydant, confiner le gaz non oxydant à l'intérieur du moule (10) et réaliser l'échappement du gaz non oxydant lors de la coulée du métal plus dense.

6. Procédé selon la revendication 5, dans lequel le moule (10) comporte des chapeaux extrêmes (22) dont au moins l'un présente un évent (24) pour l'échappement du gaz non oxydant, et comprenant l'étape qui consiste à obturer cet évent (24) pour confiner le gaz non oxydant jusqu'à la coulée du métal plus dense.

## Patentansprüche

1. Verfahren zum Zentrifugalgießen eines metallischen Gußstückes, insbesondere eines Rohres, wobei nacheinander zwei Schichten aus Metallen verschiedener Dichte und verschiedener Schmelzpunkte gegossen werden, so daß sich zwischen den beiden Schichten eine Übergangsschicht ausbildet, und zur Beendigung des Verfahrens die beiden Schichten verfestigt werden, dadurch gekennzeichnet, daß man das leichte Metall von niedrigem Schmelzpunkt, das zudem ein leicht oxidierbares Metall ist, auf den Innendurchmesser einer sich drehenden Zentrifugalgußform (10) gießt und diese Metall in der Form (10) erstarren läßt, so daß es an einem Ende der Form (10) einen dickeren Abschnitt, der sich zu einem dünneren Abschnitt verjüngt, aufweist; das dichtere und höherschmelzende Metall zunächst auf den dicken Abschnitt des verfestigten Metalls aufbringt, während die Form sich dreht, so daß es das leicht oxidierbare Metall allmählich wieder zum Schmelzen bringt und dann über deren Länge als eine Schutzschicht fortschreitet, wodurch die Oxidation des leicht oxidierbaren Metalls bei der Gießtemperatur des leichteren Metalls verhindert wird; die Zentrifugaigußform (10) weiter dreht, bis das leicht oxidierbare Metall vollständig von der Schicht bedeckt ist, und das leicht oxidierbare Metall geringerer Dichte sich radial nach innen durch das dichtere Metall bewegt, bis es den Innendurchmesser des Gießlings erreicht, wodurch verbindert wird, daß das leicht oxidierbare Metall einer unerwünschten Oxidation unterliegt, so daß ein Gießling erhalten wird, der an oder nahe seiner Außenoberfläche eine Zone (Zone 1) von hoher Konzentration an dem dichteren Metall, legiert mit einer geringen Konzentration an dem leicht oxidierbaren, leichteren Metall; eine Zone (Zone 3) mit höherer Konzentration an dem leicht oxidierbaren, leichteren Metall, die höher ist als die in Zone (1), legiert mit einer niedrigen Konzentration an dem dichteren Metall, die niedriger ist als die in Zone (1) an oder nahe an der Innenfläche; und eine Übergangszone (Zone 2) zwischen den Zonen (1 und 3), wo die Konzentration des leicht oxidierbaren, leichten Metalls kontinuierlich radial in Richtung zu der inneren Oberfläche abnimmt, aufweist.

2. Verfahren nach Anspruch 1, dadurch gekennzeichnet, daß das leicht oxidierbare, leichte und niedrig schmelzende Metall Aluminium oder eine Aluminiumlegierung ist.

3. Verfahren nach Anspruch 1 oder 2, dadurch gekennzeichnet, daß das dichtere Metall eine wärmefeste Legierung ist, die, in Gewichtsprozenten, im wesentlichen besteht aus:

4. Verfahren nach Anspruch 1, dadurch gekennzeichnet, daß das dichtere Metall ein Metall aus der Gruppe der Legierungen auf Grundlage Stahl oder Kobalt oder Legierungen auf Grundlage Nickel oder wärmefester Legierungen, die sowohl Nickel als auch Chrom enthalten, ist.

5. Verfahren nach Anspruch 1, dadurch gekennzeichnet, daß man zwischen dem Gießen des leicht oxidierbaren, leichten und niedrig schmelzenden Metalls und dem Gießen des dichteren Metalls Luft vom Innenraum der Form (10) durch ein nicht-oxidierendes Gas verdrängt, das nichtoxidierende Gas im Inneren der Form einschließt und Mittel zum Austreten des nicht-oxidierenden Gases beim Gießen des dichteren Metalls vorsieht.

6. Verfahren nach Anspruch 5, dadurch gekennzeichnet, daß die Form (10) Endkappen (22) aufweist, von denen wenigstens eine einen Gasaustrittweg (24) für den Austritt des nicht-oxidierenden Gases aufweist und daß man diesen Gasaustrittsweg (24) abdichtet, um das nichtoxidierende Gas einzuschließen, bis das Gießen des dichteren Metalls beendet ist.
